

(No Model.)

H. B. DEXTER.

CARD BOARD.

No. 372,971.

Patented Nov. 8, 1887.



FIG. 1.



FIG. 2.

WITNESSES.

Geo. M. Caley  
Henry J. Stapleton.

INVENTOR.

Henry B. Dexter.  
by Edson Salisbury Jones  
Attorney.

# UNITED STATES PATENT OFFICE.

HENRY B. DEXTER, OF PAWTUCKET, RHODE ISLAND, ASSIGNOR TO THE RHODE ISLAND CARD-BOARD COMPANY, OF SAME PLACE.

## CARD-BOARD.

SPECIFICATION forming part of Letters Patent No. 372,971, dated November 8, 1887.

Application filed June 19, 1886. Serial No. 205,672. (No model.)

*To all whom it may concern:*

Be it known that I, HENRY B. DEXTER, a citizen of the United States, residing at Pawtucket, in the county of Providence and State 5 of Rhode Island, have invented a new and useful Improvement in Card-Board; and I do hereby declare the following specification, taken in connection with the accompanying drawings forming a part of the same, to be a 10 description thereof.

This invention consists in a card-board or pasteboard, composed of several layers or sheets pasted or cemented together, the interior layer of which has incorporated or combined therewith animal hair, in a whole state, the said interior layer being covered on both 15 sides by layers or sheets which are attached thereto and seclude the interior layer from view, render the exterior of the board smooth, 20 and give said exterior a finished appearance.

In the accompanying drawings, Figure 1 shows in perspective a piece of card-board embodying the invention, with the three layers composing the same exposed to view. Fig. 25 2 represents a transverse section of the same.

The interior layer, A, of the card-board is made from pulp or material usually employed in the manufacture of paper, and there is combined therewith animal hair, *a*, in a whole 30 state, the said hair, being introduced into the pulp during the manufacture of the layer or sheet A, so as to be thoroughly incorporated with said pulp and bind the mass together. The layer A, so composed, is covered on one 35 side by a layer or sheet, B, and on the other side by a layer or sheet, C, both of ordinary paper, which sheets or layers are pasted or cemented to the layer A, thereby secluding such interior layer from view, rendering the

surface of the board smooth and giving the 40 board a finished appearance.

The incorporation or combination of hair in a whole state with the pulp or material mainly composing the layer or sheet A, binds such material more firmly together and makes the 45 layer more cohesive, thereby rendering a card-board having a layer so composed much stronger, firmer, and more durable than it otherwise would be, besides enabling the pulp or material mainly composing such layer to be 50 of a cheaper quality than if the invention were not employed.

The advantages of hair to combine with the paper-pulp are that hair being fine and smooth it will more intimately combine with the pulp 55 than other materials that have been used—such as cotton, wool, and silk—so that the surface of the board will be smoother than when threads or yarns are used. In the manufacture of the pulp having hair therein, the hair will distribute itself more uniformly through the pulp than threads or yarns would, and the hair pulp will flow more freely and evenly out upon the screens without tendency to lump or mass, thus making a more even and 60 smooth board.

What I claim as my invention, and desire to secure by Letters Patent, is—

An improved article of manufacture, card-board composed of an interior layer having 70 hair incorporated therein and exterior layers secured to said interior layer and covering the same from view, substantially as described.

HENRY B. DEXTER.

Witnesses:

EDSON SALISBURY JONES,  
HENRY J. STAPLETON.